

1

3,436,168

NEUTRAL DEVELOPING OF AZOIC COLORS  
Clemens Streck, Loudonville, N.Y., assignor to GAF Corporation, New York, N.Y., a corporation of Delaware  
No Drawing. Filed June 17, 1965, Ser. No. 464,826  
Int. Cl. D06p 5/06, 1/02

U.S. CL. 8—45

12 Claims

## ABSTRACT OF THE DISCLOSURE

A neutral developing composition and a process for employing the same, such composition comprising a coupling component, a diazo amino compound, a volatile oxygen-containing, water soluble nitrogenous organic base, and a sulfonated long chain alkyl carboxylic acid.

This invention relates to an improved process for neutral developing of azoic colors and to the compositions used therein.

More specifically, this invention relates to an improved process for neutral developing of azoic colors wherein the dyeing or printing composition contains a sulfonated long chain carboxylic acid and a water soluble nitrogenous oxygen-containing organic base.

Prior art processes for developing azoic compositions may be broadly classified into acidic developing and neutral developing.

In acidic developing the diazo compound and the coupling component are dissolved in a caustic alkali solution. The solution is thereafter made into a suitable paste by the addition of a thickening agent such as starch or gum tragacanth. After the paste is applied to the textile, as by printing, the dye is developed by exposing the textile to acidic steam. The acidic steam operates to split the diazo moiety, and the thus freed diazo couples with the coupling component to produce the color. Generally, acetic acid is used as the acid component in the steam. While acidic developing produces the desired dyed effect, attendant therewith are several disadvantages, primary of which is the offensive smell, irritating effect of the acid in the steam vapors, and corrosion of apparatus. Consequently, prior art workers have attempted to utilize a neutral steam developing process, thereby excluding the use of any acid.

Various processes for the neutral developing of azoic dyes have been utilized by prior art workers. The basic approach has been the use of an alkaline base which, after printing, evaporates on exposure to neutral steam, thereby lowering the pH and enabling the diazo to split and couple with the coupling component and subsequently produce the color. These processes include the addition to the dye preparation of organic acids, phosphoric acid and salts of acids as shown in United States Patent No. 1,951,571; the use of amine salts and amides in the print composition as illustrated in United States Patent No. 2,008,966; the replacement of caustic alkali by a volatile amine, such as diethylamine, as taught by United States Patent No. 2,125,087; and the use of an oxygen containing water-soluble nitrogenous organic base, such as diethylaminoethanol, disclosed in United States Patent No. 2,232,405.

All of the neutral developing techniques described above suffer from several disadvantages. None of the methods, for example, are satisfactory for use with slow splitting diazo compounds, such as 5-chloro-o-toluidine diazo stabilized with sarcosine, and 5-chloro-o-anisidine diazo stabilized with sarcosine. Furthermore, the shades are duller than when the same dyestuff components are developed in acid steam. The duller shades are attributable primarily to slow coupling. The pH is usually higher in

2

neutral developing than in acidic developing and therefore dissociation of the diazoamino compound is slow, coupling is slow and decomposition of diazo is high.

While this method has been found advantageous when applied to neutral developing of azoic dyes, that is by developing the color by ageing in the presence of neutral steam, it has an added feature that it is also suitable for heat developing of azoic dyes, that is by subjecting the printed or dyed fabric to a temperature of 200–425° F. to develop color. It is especially useful in the Thermosol method wherein the printed or dyed fabric is dried and then subjected to a temperature of from about 200–450° F. for from about 15 seconds to 2 minutes.

It has been found in accordance with the present invention that, by using a printing or dyeing composition containing both a sulfonated long-chain carboxylic acid and an oxygen-containing water soluble nitrogenous organic base, the disadvantages of the prior art neutral developing processes may be overcome.

In those cases where the diazoamino cleaves with great difficulty it has been found advantageous to replace part of the sulfonated long-chain carboxylic acid with a strong organic acid.

Accordingly, it is an object of this invention to provide a novel neutral developing azo dye composition and process for using the same.

Another object of this invention is to provide a neutral developing azo dye composition and process which is remarkably effective in cleaving slow-splitting diazoamino compounds.

A further object of this invention is to provide a neutral developing azo dye composition and process wherein the colors developed are as consistently as bright as that produced in the conventional acidic developing composition and process.

Another object of this invention is to provide a neutral developing azo dye composition and process which can be employed with slow-splitting diazoamino compounds which cannot be developed by the method described in United States Patent 2,232,405 which process is known as the RNA method.

Another object of this invention is to provide a composition and process wherein azoic compositions can be developed by a heat treatment.

These and other objects are accomplished by a composition containing a sulfonated long-chain carboxylic acid and a volatile water-soluble nitrogenous oxygen-containing organic base.

The volatile water-soluble nitrogenous oxygen-containing organic bases can be those recited in United States Patent No. 2,232,405, which patent is hereby incorporated by reference. Exemplary of the bases recited therein are ethylaminoethanol, diethylaminoethanol, N-propylaminoethanol, dimethylaminoethanol, dimethylaminobutanone, diethylaminoethanol methyl ether, N-hydroxyethylpyrrolidone, isobutylaminoethanol, isopropylaminoethanol and dipropylaminoethanol.

The sulfonated long-chain carboxylic acids are preferably the C<sub>12</sub> to C<sub>18</sub> sulfonated alkyl carboxylic acids such as  $\alpha$ -sulfolauric acid,  $\alpha$ -sulfotridecoic acid,  $\alpha$ -sulfomyristic acid,  $\alpha$ -sulfopentadecanoic acid,  $\alpha$ -sulfopalmitic acid,  $\alpha$ -sulfomargaric acid, and  $\alpha$ -sulfostearic acid. In addition to the  $\alpha$ -sulfonated carboxylic acids disclosed above, the term "sulfonated long-chain alkyl carboxylic acids having from 12 to 18 carbon atoms" is intended to include those compounds having one or more substituted sulfonated groups on any of the carbon atoms such as, for example, the " $\beta$ ," " $\gamma$ ," " $\delta$ ," etc., position. The choice of acid and the position and number of sulfonated groups are dependent, for the most part, on prevailing economic considerations and the availability of the particular acid utilized.

The preferred method of carrying out this invention is to combine the oxygen-containing volatile amine and sulfonated alkyl carboxylic acid to produce a composition which in turn is combined with an alkaline solution which comprises approximately equal amounts of a stabilized diazoamino compound and an azoic coupler. This solution is usually thickened with starch tragacanth, Kel-tex gum, etherified starch or similar thickeners to printing consistency, printed on the fabric and subjected to neutral steam to develop color, or if desired subjected to dry heat to develop color.

As an alternative, the amine may be added to the azoic solution followed by addition of the sulfonated alkyl carboxylic acid under agitation.

Other additives may be included in the solution such as dispersants, solvents, urea, formaldehyde and the like.

The amount of the oxygen-containing amine and sulfonated alkylcarboxylic acid may vary. It has been found, for example, that .25 to 1.5 parts of oxygen-containing amine and .01 to .5 part of sulfonated alkylcarboxylic acid, to 1 part of color component provide satisfactory results.

In those cases where the diazoamino cleaves with great difficulty it has been found that splitting is easier and faster if part of the sulfonated long-chain carboxylic acid is replaced by a strong organic acid. The strong organic acid should have an ionization constant greater than about  $1.8 \times 10^{-5}$ . In other words, the strong acid should be stronger than acetic acid. Such acids include monochloroacetic acid, glycollic acid, diglycollic acid, oxalic acid and the like. In using such acids, 5 to 50% of the sulfonated long-chain carboxylic acid is replaced in the formulations by the strong acid.

The parts indicated above and throughout the specification and claims are parts by weight.

The following examples are intended to more specifically illustrate the invention, without being limitative in any manner.

#### Example I

A developer composition of the following constituents was prepared:

|                                                | Parts |
|------------------------------------------------|-------|
| Diethylethanolamine                            | 50    |
| Diethylene glycol                              | 23    |
| $\alpha$ -Sulfostearic acid                    | 20    |
| Alipal LO-529 (sulfonated nonionic surfactant) | 7     |

An azoic solution of the following constituents was prepared.

|                                                     | Parts |
|-----------------------------------------------------|-------|
| Methyltaurine stabilized 5-chloro-o-anisidine diazo | 14.70 |
| 3-hydroxy-2-naphth-o-anisidine                      | 14.50 |
| Diethylene glycol                                   | 27.00 |
| Caustic soda flake                                  | 2.50  |

adjusted to 100 parts with water.

A print paste was prepared as follows:

|                       | Grams |
|-----------------------|-------|
| Azoic solution        | 10    |
| Urea                  | 20    |
| Developer composition | 10    |
| Starch tragacanth     | 60    |

Three swatches of cotton cloth were printed with the above paste. One swatch was dried and aged for 5 minutes with neutral steam. The second swatch was dried and treated for 3 minutes at 300° F. The third swatch was dried and treated for 1½ minutes at 425° F. All three swatches developed a full bright red color. This demonstrates color development by neutral steaming, by usual heat development and by Thermosoling.

#### Example II

Example I was repeated except that the azoic solution

was replaced by a solution prepared by mixing the following components:

|                                                 | Parts |
|-------------------------------------------------|-------|
| Sarcosine stabilized 5-chloro-o-toluidine diazo | 12.20 |
| 3-hydroxy-2-naphth-o-phenetidine                | 15.40 |
| Diethylene glycol                               | 27.00 |
| Caustic soda flake                              | 2.50  |

adjusted to 100 parts with water.

The three swatches were treated in the same manner as in Example I and each developed a full bright scarlet color.

#### Example III

A print paste was prepared as in Example I except that the azoic solution consisted of the following ingredients:

|                                                 | Parts |
|-------------------------------------------------|-------|
| Sarcosine stabilized 5-chloro-o-toluidine diazo | 11.5  |
| Bis (acetooacet) dianisidine                    | 9.0   |
| Cellosolve                                      | 20.0  |
| Caustic soda flake                              | 1.8   |

adjusted to 100 parts with water.

The three swatches were treated in the manner of Example I and each developed a bright yellow color.

#### Example IV

An azoic solution of the following constituents was prepared:

|                                                 | Parts |
|-------------------------------------------------|-------|
| Sarcosine stabilized 5-chloro-o-toluidine diazo | 15.5  |
| 3-hydroxy-2-naphth-o-toluidide                  | 16.0  |
| Diethylene glycol                               | 27.0  |
| Caustic soda flake                              | 2.5   |

adjusted to 100 parts with water.

A printing paste was prepared which consisted of:

|                                    | Parts |
|------------------------------------|-------|
| Starch tragacanth                  | 50.0  |
| Urea                               | 20.0  |
| Developer prepared as in Example I | 7.0   |
| Azoic solution prepared above      | 10.0  |
| Water                              | 13.0  |

Cotton was printed with this paste. When aged by neutral steam for 5 minutes and when subjected to heat at 300° F. for 3 minutes, bright red colors were obtained.

#### Example V

Example IV was repeated except that to the print paste was added 4.0 parts of the dispersed dye prepared by coupling 3-hydroxy-2-naphth-o-anisidine with 5-chloro-o-anisidine diazo and the water content was reduced to 9.0 parts. Dacron-cotton (65-35%) was printed with the paste, dried and cured at 400° F. for 1½ minutes. A bright red union shade was obtained.

#### Example VI

Example I was repeated except that the azoic solution was replaced by a solution prepared by combining the following components:

|                                                                           | Parts |
|---------------------------------------------------------------------------|-------|
| 2,5-dichloroaniline diazo stabilized with N-ethyl-5-sulfoanthranilic acid | 16.0  |
| 3-hydroxy-2-naphth-o-phenetidine                                          | 10.0  |
| Cellosolve                                                                | 20.0  |
| Caustic soda flake                                                        | 2.1   |

The three swatches were treated in the same manner as in Example I and each developed a bright orange color.

#### Example VII

The following printing paste was formulated:

|                                          | Parts |
|------------------------------------------|-------|
| Starch tragacanth                        | 55.0  |
| Urea                                     | 20.0  |
| Developer prepared as in Example I       | 10.0  |
| Azoic solution prepared as in Example VI | 10.0  |

Dispersed dye prepared by coupling 3-hydroxy-2-naphth-o-toluidide with 2-chloro-6-trifluoromethylaniline diazo 5.0

A 65-35% Dacron-cotton fabric was printed with this paste, dried and subjected to a temperature of 400° F. for 1½ minutes. A solid orange union shade was produced.

#### Example VIII

Example II was repeated except that the stabilized diazo was replaced by 5-chloro-o-toluidine diazo stabilized with cyanamide. 10

The three swatches were treated in the same manner as in Example I and each developed a full bright scarlet color.

#### Example IX

15

The following print paste was formulated:

|                                                 | Parts |
|-------------------------------------------------|-------|
| O/W emulsion (commercial oil-in-water emulsion) | 40.0  |
| Polygun 260 (5%) (etherified starch)            | 15.0  |
| Urea                                            | 20.0  |
| Developer prepared in Example I                 | 8.0   |
| Azoic solution prepared in Example I            | 10.0  |
| Water                                           | 7.0   |

Cotton was printed with this paste. Color was developed by curing at 400° F. for 1½ minutes and also by neutral steaming for 5 minutes. In both cases a bright bluish red color was obtained.

This formulation was modified by adding 4.0 parts of the dispersed dye prepared by coupling 3-hydroxy-2-naphth-o-toluidide with 5-chloro-o-anisidine diazo and reducing the water content to 3.0 parts.

A 65-35% Dacron-cotton fabric was printed with this paste, dried, and subjected to 400° F. for 1½ minutes. A bright red union shade was obtained.

30

35

|                                 | Examples |       |     |
|---------------------------------|----------|-------|-----|
|                                 | X        | XI    | XII |
| Parts                           | Parts    | Parts |     |
| Polygun 260 (5%)                | 50       | 50    | 50  |
| Urea                            | 20       | 20    | 20  |
| Developer of Example I          | 10       | 5     | 5   |
| The azoic solution of Example 3 | 10       |       |     |
| Azoic blue solution             |          | 10    |     |
| Azoic black solution            |          |       | 15  |
| Water                           | 10       | 10    | 10  |

40

45

The azoic blue solution consisted of:

|                                              | Parts |
|----------------------------------------------|-------|
| Methyltaurine stabilized dianisidine tetrazo | 8.5   |
| 3-hydroxy-2-naphthanilide                    | 11.0  |
| Celllosolve                                  | 5.0   |
| Diethylene glycol                            | 10.0  |
| Caustic soda flake                           | 5.0   |

50

The azoic black solution consisted of:

|                                              | Parts |
|----------------------------------------------|-------|
| Methyltaurine stabilized dianisidine tetrazo | 15.0  |
| 7 and 8-amino-5-(phenylazo)-1-naphthylamine  | 4.8   |
| 3-hydroxy-2-naphthanilide                    | 4.5   |
| Diethylene glycol                            | 10.0  |
| Caustic soda flake                           | 4.5   |

60

65

Cotton was printed with the paste of Example X, dried and subjected to a temperature of 400° F. for 1½ minutes and also a second print was steamed in neutral steam for 3 minutes. In both cases a bright yellow coloration occurred.

Two swatches of cotton were printed with the paste of Example XI. When developed as described in Example X bright blue prints were obtained.

Two swatches of cotton were printed with the paste of 75

Example XII. When developed as described in Example X deep black prints were obtained.

#### Example XIII

The following composition was formulated:

|                                                                                                  | Parts |
|--------------------------------------------------------------------------------------------------|-------|
| Urea                                                                                             | 30.0  |
| Alginate gum (1-100)                                                                             | 30.0  |
| Water                                                                                            | 50.0  |
| Developer of Example I                                                                           | 15.0  |
| Azoic solution of Example II                                                                     | 10.0  |
| Dispersed dye from 5-chloro-o-toluidine diazotized and coupled with 3-hydroxy-2-naphth-o-toluide | 8.0   |

65-35% Dacron-cotton material was padded with this solution, dried and subjected to a temperature of 400° F. for 1½ minutes. A bright solid union scarlet was obtained.

#### Example XIV

The following composition was formulated:

|                                                                                                            | Parts |
|------------------------------------------------------------------------------------------------------------|-------|
| Urea                                                                                                       | 30.0  |
| Alginate gum 1:100                                                                                         | 30.0  |
| Water                                                                                                      | 50.0  |
| Developer of Example I                                                                                     | 15.0  |
| Azoic solution of Example I                                                                                | 10.0  |
| Dispersed dye from 5-chloro-o-anisidine diazotized and coupled with 3-hydroxy-2-naphth-o-toluide           | 4.0   |
| Dispersed dye from 4-(o-tolyl-azo-o-toluidine diazotized and coupled with 3-hydroxy-2-naphth-o-phenetidine | 4.0   |

A 65-35% Dacron-cotton swatch was padded with this solution, dried and subjected to a temperature of 400° F. for 1½ minutes. A deep bluish red union color was obtained.

#### Example XV

In order to demonstrate the effectiveness of the developer of the instant invention, the azoic dye solutions utilized in Examples I thru IV were prepared in a conventional paste formulation and both neutral and acid developed.

The paste compositions were as follows:

|                           | Grams |
|---------------------------|-------|
| Stabilized dye solution   | 10.0  |
| Starch tragacanth         | 60.0  |
| 30% caustic soda solution | 1.0   |
| Water                     | 29.0  |

Four swatches of cotton cloth were printed with the above compositions. For each swatch, the paste composition was varied by using the azoic solutions of Examples I thru IV. After ageing in neutral steam for 5 minutes, it was observed that very little color developed.

However, when four identically printed swatches of cloth were exposed to acid steam for 5 minutes, a bright full color developed, commensurate with that produced when Examples I thru IV were developed in neutral steam.

This comparison clearly demonstrates the remarkable effectiveness of the developer composition of the instant invention in developing slow developing azoic dye solutions by a neutral developing technique.

#### Example XVI

A developer composition was compounded as follows:

|                      | Grams |
|----------------------|-------|
| Diethylethanolamine  | 35    |
| α-sulfopalmitic acid | 20    |

The following print pastes were made up employing the above developer composition.

|                            | Grams |      |      |      |
|----------------------------|-------|------|------|------|
| Azoic solution of Example— | 10    |      |      |      |
| I                          |       | 10   |      |      |
| II                         |       |      | 10   |      |
| III                        |       |      |      | 10   |
| IV                         |       |      |      |      |
| Alginate gum (5%)          | 58.5  | 58.5 | 58.5 | 58.5 |
| Urea                       | 20    | 20   | 20   | 20   |
| Developer composition      | 8     | 8    | 8    | 8    |

Three swatches of cotton cloth were printed with each of the four pastes. One set was dried and aged 5 minutes in neutral steam, one set was dried and heated to 300° F. for 3 minutes, the third set was dried and heated to 425° F. for 1½ minutes. In each case, full bright color developed.

#### Example XVII

Example XVI was repeated except that the developer composition of the following composition was utilized:

|                     | Grams |
|---------------------|-------|
| Diethylethanolamine | 35    |
| α-Sulfolauric acid  | 20    |

In each case a full bright color developed.

#### Example XVIII

The following formulation was prepared:

|                                                                           | Parts |
|---------------------------------------------------------------------------|-------|
| Diethylethanolamine                                                       | 50.0  |
| Diethyleneglycol                                                          | 23.0  |
| Emulphor ELA (polyoxylated vegetable oil, General Aniline and Film Corp.) | 7.0   |
| α-Sulfostearic acid                                                       | 13.0  |
| Glycollic acid                                                            | 7.0   |

A print paste was made in the manner of Example I except that the developer solution of Example I was replaced by this solution.

Three swatches of cloth were treated as in Example I. The color produced was commensurate with that produced in Example I; however the color developed quicker.

What is claimed is:

1. A dye composition comprising coupling components, diazoamino compounds, volatile oxygen-containing, water-soluble nitrogenous organic bases and sulfonated long-chain alkyl carboxylic acids.

2. A composition according to claim 1, wherein the sulfonated long-chain alkyl carboxylic acid has from 12 to 18 carbon atoms.

3. A composition according to claim 1, wherein the sulfonated long-chain alkyl carboxylic acid is α-sulfolauric acid.

4. A composition according to claim 1, wherein the sulfonated long-chain alkyl carboxylic acid is α-sulfo-palmitic acid.

5. A composition according to claim 1, wherein the sulfonated long-chain alkyl carboxylic acid is α-sulfo-stearic acid.

10 6. In the method of neutral steam developing of azoic dyes, the improvement which comprises applying to the material to be dyed a developer composition comprising coupling components, diazoamino compounds, volatile nitrogenous oxygen-containing organic bases, and sulfonated long-chain alkyl carboxylic acid.

7. The method according to claim 6, wherein the sulfonated long-chain alkyl carboxylic acid has from 12 to 18 carbon atoms.

15 8. The method according to claim 6, wherein the sulfonated long-chain alkyl carboxylic acid is α-sulfolauric acid.

9. The method according to claim 6, wherein the sulfonated long-chain alkyl carboxylic acid is α-sulfopalmitic acid.

10 10. The method according to claim 6, wherein the sulfonated long-chain alkyl carboxylic acid is α-sulfostearic acid.

11 11. A composition according to claim 1 wherein 5 to 50% by weight of the sulfonated long-chain alkyl carboxylic acid is replaced by a strong organic acid having an ionization constant of at least  $1.80 \times 10^{-5}$ .

12 12. A method according to claim 6 wherein 5 to 50% by weight of the sulfonated long-chain alkyl carboxylic acid is replaced by a strong organic acid having an ionization constant of at least  $1.80 \times 10^{-5}$ .

#### References Cited

##### UNITED STATES PATENTS

2,232,405 2/1941 Schmelzer ----- 8—45

NORMAN G. TORCHIN, Primary Examiner.

T. J. HERBERT, Jr., Assistant Examiner.

U.S. Cl. X.R.

45 8—46